

Aug. 14, 1945.

O. A. J. VAN LIN ET AL

2,382,275

INSULATED ELECTRIC CONDUCTOR

Filed April 8, 1941



Inventors:

O. A. J. VAN LIN  
J. HOEKSTRA

*By Allentown  
Attorney.*

## UNITED STATES PATENT OFFICE

2,382,275

## INSULATED ELECTRIC CONDUCTOR

Oswaldus Anthonius Jacobus van Lin, Venlo, and  
 Johannes Hoekstra, Eindhoven, Netherlands;  
 vested in the Alien Property Custodian

Application April 8, 1941, Serial No. 387,508  
 In the Netherlands April 11, 1940

2 Claims. (Cl. 117—78)

To make use of insulating layers consisting either of rubber hydrochloride or containing rubber hydrochloride as a chief constituent for insulating electric conductors is known.

Such insulating layers which can be easily made by means of the material commercially known as "Pliofilm" have excellent electric properties; moreover, they are elastic and have a particularly great mechanical strength. Such an insulating layer may be applied in form of an envelope, for instance by wrapping the material, in the form of a band, about the conductor and then heating so the windings stick together.

In spite of the fact that these insulating layers are also impermeable to water such an insulating layer is often insufficient without the intervention of other means because of the loss of the excellent electric properties upon contact with water when the disruptive strength may decrease to 0.1 of the initial value and the electric resistance drop appreciably.

The present invention has for its object to avoid this drawback in order that the particular properties of the insulating layers in question may be utilized as much as possible.

To this end, the insulating layer consisting of rubber hydrochloride or containing rubber hydrochloride as a chief constituent is, according to the invention, coated with an insulating layer which entirely or substantially entirely consists of chlorinated rubber containing more than 60% by weight of chlorine. Such a layer, which can be easily applied in the form of a solution of lacquer, has the advantage over other layers impermeable to water of being very impermeable and resistant to water and possessing excellent electrical properties such as break-down voltage, insulation resistance and dielectric losses.

However, a drawback arises in that the layer of chlorinated rubber is very sensitive to temperature variations particularly with regard to its mechanical properties, so that it is very difficult to make a layer which is not brittle at low temperatures and sticky or soft at high temperatures.

Therefore, in one form of carrying the invention into effect, the layer of chlorinated rubber impermeable to water may be covered with an elastic layer having a great mechanical strength at low and high temperatures. Such a layer can be obtained in known manner by applying it in form of a solution of cellulose lacquer followed by drying; as an alternative this may be effected by making use of a layer of rubber hydrochloride.

Moreover, a greater rigidity and ductility of the

whole of the insulating layer is obtained according to this executional example.

For making the invention better understood it may still be observed that directly coating the insulating layer of rubber hydrochloride with the elastic layer having a great mechanical strength referred to above does not yield the results obtained according to the invention, because such layers generally do not approximate the impermeability or resistance to water of the said layer of chlorinated rubber.

In order that the invention may be clearly understood and readily carried into effect, we shall describe the same in more detail with reference to the accompanying drawing in which the single figure is a partly-sectionized view of a cable according to the invention.

The cable shown in the drawing comprises a stranded conductor consisting of six steel wires 1 of 0.35 mm. in diameter and two copper wires 2—22 of 0.35 and 0.5 mm. in diameter respectively, twice wrapped in opposite sense with a film 3 of rubber hydrochloride (e. g. "Pliofilm") having a width of 2.5 mm. and a thickness of 0.03 mm. This envelope is fused together by heating for a short time at 110 to 120° C. and then coated with a layer 4 consisting, for instance, of 33% by weight of tricresylphosphate and 67% by weight of chlorinated rubber having a high viscosity. This layer may be provided in several layers by painting a solution e. g. in benzene by means of a nozzle followed by drying of the whole layer which is preferably effected by raising the temperature stepwise or continuously during this drying operation. On to this layer 5 is applied a layer of lacquer consisting, for instance, of 57% by weight of acetylcellulose, 13% by weight of triphenylphosphate and 30% by weight of tributylphosphate which is followed by drying also this layer. After that the wire thus insulated may still be covered in a known manner with a flax braiding (not shown) which may be coated in known manner with a compound containing asphalt bitumen (not shown).

The invention is of particular importance for weak current conductors destined for non-permanent telephonic and telegraphic connections where use is often made of a core usually consisting of a plurality of single metal wires, which core has a high tensile strength, for instance of more than 75 kg./mm.<sup>2</sup> and requires a thin, light and strong insulating envelope having a high insulation resistance, as can be obtained according to the invention.

## What we claim is:

1. An insulated electric cable comprising a conductor, an insulating layer surrounding said conductor and formed mainly of rubber hydrochloride, and an insulating layer covering said first layer and formed mainly of chlorinated rubber containing more than 60% by weight of chlorine.

2. An insulated electric conductor as claimed in claim 1, comprising in addition a third insulating layer which is elastic and has a great mechanical strength at low and high temperatures, for instance, consisting of cellulose lacquer.  
OSWALDUS ANTHONIUS JACOBUS VAN LIN.  
JOHANNES HOEKSTRA.